# EUROPEAN PATENT SPECIFICATION

(11) **EP 0 613 938 B1**
(45) Date of publication and mention of the grant of the patent: **22.07.1998**
(21) Application number: 94301303.7
(22) Date of filing: 24.02.1994
(51) Int. Cl.: C10L 1/22

(54) **Hydrocarbon fuel compositions incorporating nitrogen-containing dispersants**
Stickstoff enthaltende Dispergiermittel umfassende Kohlenwasserstoffkraftstoffszusammensetzungen
Compositions de combustible hydrocarboné incorporant des dispersants contenant de l'azote

(30) Priority: 03.03.1993 GB 9304350
(43) Date of publication of application: 07.09.1994
(73) Proprietor: BP Chemicals (Additives) Limited, Hemel Hempstead, Hertfordshire HP2 4UL (GB)
(72) Inventor: Clarke, Michael John, Hedon, Hull HU12 8DS (GB); Duncan, David Anthony, Hedon, Hull HU12 8DS (GB)
(74) Representative: Preece, Michael

(56) References cited:
- EP-A- 0 062 161
- EP-A- 0 191 967
- EP-A- 0 208 560
- FR-A- 2 197 062
- GB-A- 1 378 708
- GB-A- 1 471 601
- US-A- 3 324 033
- US-A- 4 234 435
- DATABASE WPI Week 7637, Derwent Publications Ltd., London, GB; AN 76-69240X & JP-A-50 051 985 (TOA NENRYO KOGYO KK)

## Description

The present invention relates in general to internal combustion engine fuel compositions. In particular the invention relates to the use of nitrogen-containing compounds as dispersants in the aforesaid fuel compositions.

The use of nitrogen-containing compounds for the purpose of maintaining sludge-forming deposits dispersed in internal combustion engine lubricating oils, thereby keeping the piston and piston rings relatively free of deposits, is well known. Nitrogen-containing compounds which have long been used as dispersant/detergent additives in lubricating oils include the hydrocarbyl-substituted succinimides. The preparation of succinimides and their use as lubricating oil additives is described in, for example, US-A-3,024,237; US-A-3,202,678; US-A-3,219,666 and US-A-3,275,554.

Hydrocarbon fuels generally contain numerous deposit-forming substances. When used in internal combustion engines, deposits tend to form on and around constricted areas of the engine in contact with the fuel. In diesel engines, deposits tend to accumulate in the fuel injection system, thereby hampering good performance of the engine. In automobile engines deposits can build up on engine intake valves leading to progressive restriction of gaseous fuel mixture flow into the combustion chamber and also to valve sticking. It is common practice to incorporate a detergent in the fuel composition for the purpose of inhibiting the formation, and facilitating the removal, of engine deposits, thereby improving engine performance. Nitrogen-containing compounds commonly used as additives in hydrocarbon fuels include polyisobutene amines. Their use is described in, for example, US-A-3,565,804; US-A-3,756,793; and US-A-4,877,416. Polyisobutene succinimides have also been disclosed as hydrocarbon fuel additives in, for example, EP-A-0147240.

Although there are references in the prior art to the use of polyisobutene succinic amide-containing materials as additives to fuel compositions, there would not appear to be any specific mention in this context of the use of hydrocarbyl-substituted succinic diamides obtainable by reacting at elevated temperature a hydrocarbyl-substituted succinic acid or an anhydride, ester or monoamide derivative thereof with a secondary amine. Thus, US-A-3,236,613 discloses petroleum distillate hydrocarbon fuels containing from between about 1 to about 100 pounds, per thousand barrels of fuel, of a compound of the following formula: wherein R is the aliphatic residue of an aliphatic dicarboxylic acid, R' is an aliphatic hydrocarbon group, R'' is a member from the group consisting of and x is an integer from 1 to 6. Such compounds can be prepared by heating at 75 to 100ºC for about 2 hours a mole to mole mixture of an aliphatic dicarboxylic acid anhydride and aliphatic primary amine to form the amic acid, ie subjecting the amic acid (A) to condensation reaction at 95ºC to 150ºC for 2 to 5 hours with a polyamine of the following formula:

(R'')ₓNH₂

in substantially molar amounts to provide the following condensation reaction product: and further condensing product (B) in mole to mole ratio with salicyladehyde at 125 to 175ºC for 2 to 5 hours. The compounds function as anti-screen clogging and sediment stabilising addiion agents for petroleum hydrocarbon distillate fuel oils and, as antioxidants and metal deactivators in both fuel oils and gasolines. Other publications, eg US-A-4,698,169 and EP-A-191967 disclose a reaction product useful as either a fuel or lubricant additive which is obtained by the reaction of an alkenyl succinic anhydride or acid with an aromatic secondary amine to form an intermediate product and thereafter reacting the intermediate product with either an alkanolamine, an aminomethane or a hindered alcohol.

We have now found that the hydrocarbyl-substituted succinic diamides obtainable as described hereinafter are particularly useful as dispersants in fuel compositions.

Accordingly in one aspect the present invention provides a hydrocarbon fuel composition comprising a hydrocarbon fuel and an amount sufficient to provide dispersancy of a hydrocarbyl-substituted succinic diamide, wherein the hydrocarbyl substituent is of a size sufficient to render the diamide soluble in the fuel, the diamide being obtainable by reacting at elevated temperature a secondary amine with either a hydrocarbyl-substituted succinic acid or an anhydride, ester or monoamide derivative thereof.

The hydrocarbyl substituent of the succinic diamide is of a size sufficient to render the diamide soluble in the hydrocarbon fuel. Typically this may be achieved with a hydrocarbyl substituent having at least 25 carbon atoms, preferably greater than 35 carbon atoms, and up to about 500 carbon atoms, preferably up to about 300 carbon atoms. The hydrocarbyl substituent may be derived from a suitable polyalkene or mixture of polyalkenes selected from, for example, polyethylene, polypropylene and polybutenes. A preferred hydrocarbyl substituent is derived from a polyisobutene. Polyisobutene succinic anhydrides (PIBSAs) suitable for use in the reaction may be obtained commercially. They are generally prepared by reacting maleic anhydride with a polyisobutene by either a thermal or a chlorination route. An advantage of the thermal route for the preparation of PIBSAs is that it minimises contamination of the PIBSA with residual chlorine. Polyisobutene succinic acids suitable for use in the reaction may be obtained by hydrolysis of PIBSAs, suitably using water as the hydrolysing agent, and at elevated temperature. Polyisobutene succinic acid esters may suitably be obtained by esterification of either a PIBSA or a polyisobutene succinic acid. Polyisobutene succinic monoamides may suitably be obtained by reacting a PIBSA or a polyisobutene succinic acid salt with up to 1 mole per mole of a secondary amine.

As the secondary amine there may be used a secondary mono-, di- or poly-amine. Thus there may be used a secondary mono-amine having the formula:- wherein R¹ and R² are independently C₁-C₁₅ hydrocarbyl groups, suitably alkyl groups, preferably C₁ to C₄ alkyl groups. Alternatively, there may be used a secondary diamine having the formula:- wherein X is a divalent hydrocarbyl group, suitably an alkylene group, having up to 15 carbon atoms, preferably up to 6 carbon atoms; and R¹ and R² are independently C₁ to C₁₅ hydrocarbyl groups, suitably alkyl groups, preferably C₁ to C₄ alkyl groups. Alternatively, there may be used a secondary polyamine having the formula:- wherein X is a C₁ to C₁₅ divalent hydrocarbyl group, suitably a C₁ to C₆ alkylene group, preferably an ethylene or propylene group, which may be substituted with, for example, hydroxyl groups; R¹ and R² are independently C₁ to C₁₅ hydrocarbyl groups, suitably alkyl groups, preferably C₁ to C₄ alkyl groups; and n is an integer in the range from 1 to 6, preferably from 1 to 4. Preferred secondary amines include dialkanolamines of the formula:-

(HOR¹)₂NH (IV)

wherein R¹ = C₁ to C₆ alkylene, for example ethylene; derivatives thereof having the formula:-

(HOR¹[NHR²]ₙ)₂NH (V)

wherein R¹ and R² are independently C₁ to C₆ alkylene, for example ethylene, and n is an integer in the range from 1 to 6, for example 1; and N-alkyl piperazines of the formula:- wherein R² is an alkyl group, suitably a C₁ to C₁₀ alkyl group, for example methyl, ethyl, propyl or butyl. Of these, N-alkyl piperazines are preferred because they eliminate the possibility of the diamide product being contaminated with esters, unlike compounds of the formulae (IV) and (V). A preferred secondary amine reactant is N-methyl piperazine.

The hydrocarbyl-sutstituted succinic diamide is obtainable by reacting at elevated temperature a hydrocarbyl-substituted succinic acid or an anhydride, ester or monoamide derivative thereof with a secondary amine. The reactants are reacted in proportions such that there is formed a diamide. Using a hydrocarbyl-substituted succinic acid or anhydride it is preferred to react at least 2 moles of the secondary amine for each mole of acid or anhydride. Using a hydrocarbyl-substituted succinic acid monoamide it is preferred to react at least 1 mole of the secondary amine for each mole of monoamide. It is preferred to react a hydrocarbyl substituted succinic acid or anhydride with at least 2 moles of the secondary amine for each mole of acid or anhydride. Using a hydrocarbyl-substituted succinic acid monoamide as the starting material for the reaction with the secondary amine it is possible to produce diamides having different amido substituents by employing a secondary amine different to that used in the formation of the monoamide. Otherwise mixtures of diamides may be obtainable by using mixtures of at least two secondary amines in the diamide forming reaction.

The reaction may be accomplished in the presence or absence of a solvent. Suitable solvents include liquid hydrocarbons, for example xylene or cyclohexane.

The reaction of the acid or derivative thereof with the secondary amine may suitably be effected at elevated temperatures, suitably below 250°C, for example from about 90 to 180°C. The reaction of a PIBSA with diethanolamine, for example, may suitably be represented as follows:-

The reaction of a polyisobutene succinic acid with N-methyl piperazine, for example, may suitably be represented as follows:

The hydrocarbon fuel may suitably comprise a hydrocarbon fraction boiling in the gasoline range or a hydrocarbon fraction boiling in the diesel range. Gasolines suitable for use in spark ignition engines, eg automobile engines, generally boil in the range from 30 to 230°C. Such gasolines may comprise mixtures of saturated, olefinic and aromatic hydrocarbons. They may be derived from straight-run gasoline, synthetically produced aromatic hydrocarbon mixtures, thermally or catalytically cracked hydrocarbon feedstocks, hydrocracked petroleum fractions or catalytically reformed hydrocarbons. The octane number of the base fuel is not critical and will generally be above 65. In the gasoline, hydrocarbons may be replaced in part by alcohols, ethers, ketones or esters, typically in an amount up to 20% by weight. Alternatively, as the liquid hydrocarbon fuel there may be used any fuel suitable for operating spark compression engines, such as those which may be found in road vehicles, ships and the like. Generally, such a diesel fuel will boil in the range from about 140°C to about 400°C (at atmospheric pressure), particularly in the range from about 150 to 390°C, especially from about 175 to 370°C. Such fuels may be obtained directly from crude oil (straight-run) or from a catalytically or thermally cracked product or a hydrotreated product, or from a mixture of the aforesaid. Alternatively there may be used a biofuel, for example rape seed methyl ester. The cetane number will typically be in the range from 25 to 60.

The fuel composition contains the hydrocarbyl substituted succinic diamide in an amount sufficient to provide dispersancy. Typically in a gasoline fuel this amount will be in the range from 20 to 1000 ppm w/w based on the total weight of the composition. Typically in a diesel fuel this amount will be in the range from 10 to 500 ppm w/w based on the total weight of the composition.

The fuel composition may suitably be prepared by blending a concentrate composition comprising a fuel compatible hydrocarbon solvent and the hydrocarbyl-substituted succinic diamide with the hydrocarbon fuel.

The fuel composition in addition to the hydrocarbyl-substituted succinic diamide may contain known additives. The nature of the additives will depend to some extent on the end-use of the fuel composition. Diesel fuel compositions may contain nitrates or nitrites as a cetane improver, or copolymers of ethylene and/or vinylesters, eg vinylacetate, as a pour point depressant. Gasoline fuel compositions may contain a lead compound as an anti-knock additive and/or an antioxidant, eg 2,6-di-tert-butyl phenol, and/or an anti-knock compound other than a lead compound, and/or an additional dispersant, for example a PIB polyamine. The other additives (if any) may be blended directly into the fuel composition or may be incorporated by way of a concentrate composition.

The invention will now be further illustrated by reference to the following examples.

### EXAMPLE A

### Preparation of "Clean" polyisobutenyl succinic anhydride (PIBSA) for subsequent diamide preparations

A blend of 2 kg PIBSA (produced by the thermal maleinisation of a polyisobutene (PIB) of number average molecular weight (Mₙ) of about 1000) and 500 g of n-heptane was prepared. This was heated to about 80^{º}C and then filtered through a diatomaceous earth filter aid. The filtration temperature was maintained at 50-60ºC by the use of heat lamps.

The n-heptane was subsequently removed on a rotary evaporator at 110ºC/28 inches Hg over one hour.

Some maleic anhydride (MA) was removed on the strip stage as evidenced by the condenser coils "furring up" with crystals.

Data from the determination of the residual MA and PIBSA No. (mg KOH/equivalent/g) of the various PIBSAs is given in the following Table 1.

**TABLE 1**

| **PIBSA** | **MA(%)** | **PIBSA No.** |
|---|---|---|
| PIBSA | 0.3 | 103 |
| PIBSA 80/20 with n-heptane | 0.1 | 84 |
| PIBSA, diluted, filtered and stripped ie "clean" | less than 0.05 | 101.5 |

### Example 1

### Preparation of Diamide

N-methyl piperazine (NMP)(25 g), the "clean" PIBSA of Example A (200 g) and xylene (100 g) were mixed and the mixture heated to reflux at 165-170ºC. The mixture was held at the reflux temperature for 3 hours.

| Water Evolution | |
|---|---|
| Up to 3 hours | about 1.0 ml. |
| End of reaction | about 1.2 ml. |

| Solvent Removal | |
|---|---|
| Charged | 312.7 g. |
| Product wt. | 207.9 g. |

The product was stripped on a rotary evaporator at 130ºC/29.5 inches Hg.

| Analysis of Product | |
|---|---|
| Total nitrogen | 2.8%. |
| Basic nitrogen | 1.6%. |
| Alkalinity value | 65.3 mg KOH/g. |

### Example 2

### Preparation of diamide

The "clean" PIBSA of Example A (200 g), xylene (100 g) and water (3.3 g) were mixed and heated to 90ºC. After one hour N-methyl piperazine (NMP) (25 g) was added and the mixture heated to reflux at 165-170ºC, peaking at 173ºC after 4½ hours.

| Water Removal | |
|---|---|
| Time Elapsed | Water Removed |
| 80 minutes (173ºC) | 4.0 ml |
| 360 minutes (end) | 5.6 ml |

| Solvent Strip | |
|---|---|
| Charge | 304 g. |
| Product wt | 219.1 g. |

The product was stripped on a rotary evaporator at 130ºC/28 inches Hg.

| Analysis of Product | |
|---|---|
| Total nitrogen | 2.8% |
| Basic nitrogen | 1.6% |
| Alkalinity value | 62.7 mg KOH/g |

### Example 3

### Preparation of diamide

Example 2 was repeated except that instead of using xylene (100 g) there was used cyclohexane (100 g). In this preparation vigorous reflux occurred initially. A temperature of 107ºC was attained. After removal of 16.8 g cyclohexane a reflux temperature of 140ºC was attained.

| Water Removal | |
|---|---|
| Time Elapsed | Water Removed |
| 65 minutes (107ºC) | 1.5 ml |
| 345 minutes (end) | 4.6 ml |

| Solvent Strip | |
|---|---|
| Charge | 271.3 g. |
| Product wt | 206.2 g. |

The product was stripped on a rotary evaporator at 130ºC/28 inches Hg.

| Analysis of Product | |
|---|---|
| Total nitrogen | 2.7% |
| Basic nitrogen | 1.7% |
| Alkalinity value | 66.6 mg KOH/g |

### Example 4

### Preparation of diamide

A "clean" PIBSA derived from a commercially available more reactive, ie higher vinylidene content (about 60%) PIB of Mₙ about 1300 was obtained by blending the PIBSA (715 g) and n-heptane (185 g) followed by filtering through a diatomaceous earth filter aid and removing the n-heptane solvent by rotary evaporation at 130ºC/28 inches Hg (425 g blend charged; 400.1 g product recovered).

"Clean" PIBSA obtained as described above (202.9 g), xylene (100 g) and water (3.6 g) were mixed and held at 90ºC for one hour to hydrolyse the PIBSA. N-methylpiperazine (NMP) (25 g) was then added and the mixture heated to 165-170ºC at which point reflux commenced. A total of 4 hours reaction time was allowed before the product was stripped on the rotary evaporator at 130ºC/28 inches Hg (charge 322.1 g; product wt. 220.1 g).

| Analysis of Product | |
|---|---|
| Total nitrogen | 2.3%. |
| Basic nitrogen | 1.4%. |
| Alkalinity value - | 55.2 mg KOH/g. |

### Example 5

### Preparation of diamide

N-methylpiperazine (NMP) (60 g) (b.pt. 138ºC) was added dropwise to a solution of commercially available PIBSA (75% solution derived from PIB of Mₙ about 1000 in an aromatic solvent)(400 g) in xylene (100 g) at 90-120ºC over 15 minutes. An extra 100 g of xylene was added to stimulate reflux. Water (10 g) was added to hydrolyse the PIBSA. The temperature was then increased to reflux. Solvent was removed at 28 inches Hg/150ºC.

| Analysis of Product | Observed |
|---|---|
| Total nitrogen | 2.2% |
| Basic nitrogen | 1.2% |
| Alkalinity value | 45.9 |

### Example 6

### Preparation of diamide

A mixture of a PIBSA identical to that used in Example 5 (400 g), xylene (230 g) and water (6.2 g) was charged to a one litre 5-necked flange pot reactor equipped with Eurotherm, agitator and Dean and Stark trap. The contents were then heated to 95ºC to effect hydrolysis. Subsequently N-methyl piperazine (NMP) (64.8 g; b.pt. 138ºC) was added.

The product was stripped at 150ºC/28.5 inches Hg to remove solvents.

| Analysis of product | |
|---|---|
| Total nitrogen | 2.4%. |
| Basic nitrogen | 1.5%. |
| Alkalinity value | 59.5 mg KOH/g. |

### Example 7

### Preparation of diamide

A mixture of a PIBSA identical to that used in Example 5 (400g), xylene (250g) and water (6.0g) was charged to a one litre 5-necked flange pot reactor equipped with Eurotherm, agitator and Dean and Stark trap. The contents were heated to 95°C and reacted for 2 hours prior to addition of N-methylpiperazinc (65.3g).

The product was stripped at 150°C/28.5 inches Hg.

| Analysis of product | |
|---|---|
| Total nitrogen | 2.4%. |
| Basic nitrogen | 1.3%. |
| Alkalinity value | 51.2mg KOH/g. |

### Example 8

### Engine testing of diamide product

Results were generated in an Opel Kadett engine test run on fuel treated with either 500 or 1000 ppm w/w of an additive package. The additive package was based on a commercial formulation modified in the respect that the customary dispersant actives component was replaced on a weight/weight basis in turn by a dispersant according to the invention and prior art succinimide dispersants as indicated in Table 2 below. In Table 2 reference is made to succinimides 1 and 2. These materials are characterised as follows:-
Succinimide 1 is a mono-succinimide derived from an oil-free PIBSA identical to that used in Example 5, the amine used in the preparation being tetraethylenepentamine (TEPA).
Succinimide 2 is a bis-succinimide derived from an oil-free PIBSA identical to that used in Example 5, the amine used in the preparation being triethylenetetramine (TETA).

**TABLE 2**

| **Disperant Used** | **Package Treat (ppm) w/w** | **Deposits mg/Valve** | **Manifold Rating** | **Valve Rating** |
|---|---|---|---|---|
| Diamide (product of Ex. 7) | 500 | 13 | 7.88 | 9.90 |
| Diamide (product of Ex. 7) | 1000 | 6 | 8.95 | 10.0 |
| Succinimide 1 | 500 | 229 | 10.0 | 8.0 |
| Succinimide 2 | 1000 | 40 | 9.87 | 9.70 |

It can be seen from the results presented in Table 2 that the diamide product of the invention is superior in most respects to comparable succinimide dispersants in the Opel Kadett engine test.

## Claims

1. A hydrocarbon fuel composition comprising a hydrocarbon fuel and an amount sufficient to provide dispersancy of a hydrocarbyl-substituted succinic diamide, wherein the hydrocarbyl substituent is of a size sufficient to render the diamide soluble in the fuel, the diamide being obtainable by reacting at elevated temperature a secondary amine with either a hydrocarbyl-substituted succinic acid or an anhydride, ester or monoamide derivative thereof.

2. A hydrocarbon fuel composition according to claim 1 wherein the hydrocarbyl substituent has from 35 to 300 carbon atoms.

3. A hydrocarbon fuel composition according to either claim 1 or claim 2 wherein the hydrocarbyl substituent is derived from a polyisobutene.

4. A hydrocarbon fuel composition according to any one of the preceding claims wherein the secondary amine reacted with the hydrocarbyl-substituted succinic acid or derivative thereof is a dialkanolamine of the formula:-
(HOR¹)₂NH (IV)
wherein R¹ is a C₁ to C₆ alkylene group.

5. A hydrocarbon fuel composition according to any one of claims 1 to 3 wherein the secondary amine reacted with the hydrocarbyl-substituted succinic acid or derivative thereof is of the formula:-
(HOR¹ [NHR²]ₙ)₂NH (V)
wherein R¹ and R² are independently C₁ to C₆ alkylene groups and n is an integer in the range from 1 to 6.

6. A hydrocarbon fuel composition according to any one of claims 1 to 3 wherein the secondary amine reacted with the hydrocarbyl-substitued succinic acid or derivative thereof is an N-alkyl piperazine of the formula: wherein R² is a C₁ to C₁₀ alkyl group.

7. A hydrocarbon fuel composition according to claim 6 wherein the N-alkyl piperazine is N-methyl piperazine.

8. A hydrocarbon fuel composition according to any one of claims 1 to 7 wherein the hydrocarbyl-substituted succinic acid or derivative thereof is reacted with the secondary amine at a temperature in the range from 90 to 180^{º}C.

9. A hydrocarbon fuel composition according to any one of the preceding claims wherein the hydrocarbon fuel comprises a hydrocarbon fraction boiling in the gasoline range.

10. A hydrocarbon fuel composition according to any one of claims 1 to 8 wherein the hydrocarbon fuel comprises a hydrocarbon fraction boiling in the diesel range.

## Patentansprüche

1. Kraftstoffzusammensetzung, umfassend einen Kohlenwasserstoffkraftstoff und eine zur Bereitstellung von Dispergiervermögen ausreichende Menge eines Kohlenwasserstoff-substituierten Bernsteinsäurediamids, wobei der Kohlenwasserstoffsubstituent von ausreichender Größe ist, um das Diamid in dem Kraftstoff löslich zu machen, wobei das Diamid durch Umsetzen eines sekundären Amins mit entweder einer Kohlenwasserstoff-substituierten Bernsteinsäure oder einem Anhydrid, Ester oder Monoamidderivat davon bei hoher Temperatur erhältlich ist.

2. Kohlenwasserstoff-Kraftstoffzusammensetzung nach Anspruch 1, wobei der Kohlenwasserstoffsubstituent 35 bis 300 Kohlenstoffatome aufweist.

3. Kohlenwasserstoff-Kraftstoffzusammensetzung nach entweder Anspruch 1 oder Anspruch 2, wobei der Kohlenwasserstoffsubstituent von einem Polyisobuten abgeleitet ist.

4. Kohlenwasserstoff-Kraftstoffzusammensetzung nach einem der vorangehenden Ansprüche, wobei das sekundäre Amin, das mit der Kohlenwasserstoff-substituierten Bernsteinsäure oder einem Derivat davon umgesetzt wird, ein Dialkanolamin der Formel:
(HOR¹)₂NH (IV),
worin R¹ eine C₁- bis C₆-Alkylengruppe darstellt, ist.

5. Kohlenwasserstoff-Kraftstoffzusammensetzung nach einem der Ansprüche 1 bis 3, wobei das sekundäre Amin, das mit der Kohlenwasserstoff-substituierten Bernsteinsäure oder einem Derivat davon umgesetzt wird, die Formel:
(HOR¹ [NHR²]ₙ)₂NH (V),
worin R¹ und R² unabhängig C₁- bis C₆-Alkylengruppen darstellen und n eine ganze Zahl im Bereich von 1 bis 6 ist, aufweist.

6. Kohlenwasserstoff-Kraftstoffzusammensetzung nach einem der Ansprüche 1 bis 3, wobei das sekundäre Amin, das mit der Kohlenwasserstoff-substituierten Bernsteinsäure oder einem Derivat davon umgesetzt wird, ein N-Alkylpiperazin der Formel: worin R² eine C₁- bis C₁₀-Alkylgruppe darstellt, ist.

7. Kohlenwasserstoff-Kraftstoffzusammensetzung nach Anspruch 6, wobei das N-Alkylpiperazin N-Methylpiperazin ist.

8. Kohlenwasserstoff-Kraftstoffzusammensetzung nach einem der Ansprüche 1 bis 7, wobei die Kohlenwasserstoff-substituierte Bernsteinsäure oder das Derivat davon mit dem sekundären Amin bei einer Temperatur im Bereich von 90 bis 180°C umgesetzt wird.

9. Kohlenwasserstoff-Kraftstoffzusammensetzung nach einem der vorangehenden Ansprüche, wobei der Kohlenwasserstoffkraftstoff eine Kohlenwasserstofffraktion, die im Benzinbereich siedet, umfaßt.

10. Kohlenwasserstoff-Kraftstoffzusammensetzung nach einem der Ansprüche 1 bis 9, wobei der Kohlenwasserstoffkraftstoff eine Kohlenwasserstofffraktion, die im Dieselbereich siedet, umfaßt.

## Revendications

1. Composition de carburant hydrocarboné comprenant un carburant hydrocarboné et une quantité suffisante pour procurer une dispersibilité d'un diamide succinique substitué par un hydrocarbyle, dans laquelle le substituant hydrocarbyle est d'une taille suffisante pour rendre le diamide soluble dans le carburant, diamide que l'on peut obtenir en faisant réagir, à température élevée, une amine secondaire soit avec un acide ou un anhydride succinique substitué par un hydrocarbyle soit avec un dérivé ester ou monoamide de ceux-ci.

2. Composition de carburant hydrocarboné selon la revendication 1, dans laquelle le substituant hydrocarbyle possède de 35 à 300 atomes de carbone.

3. Composition de carburant hydrocarboné selon l'une des revendications 1 ou 2, dans laquelle le substituant hydrocarbyle est dérivé d'un polyisobutène.

4. Composition de carburant hydrocarboné selon l'une des revendications précédentes, dans laquelle l'amine secondaire qui réagit avec l'acide succinique substitué par un hydrocarbyle ou un dérivé de celui-ci est une dialcanolamine de formule:
(HOR¹)₂NH (IV)
dans laquelle R¹ représente un groupe alkylène en C₁ à C₆

5. Composition de carburant hydrocarboné selon l'une des revendications 1 à 3, dans laquelle l'amine secondaire qui réagit avec l'acide succinimique ou un dérivé de celui-ci a la formule
(HOR¹ [NHR²]ₙ)₂NH (V)

6. Composition de carburant hydrocarboné selon l'une des revendications 1 à 3, dans laquelle l'amine secondaire qui réagit avec l'acide succinique substitué par un hydrocarbyle ou un dérivé de celui-ci est une N-alkyl-pipérazine de formule dans laquelle R² représente un groupe alkyle en C₁ à C₁₀.

7. Composition de carburant hydrocarboné selon la revendication 6, dans laquelle la N-alkylpipérazine est la N-méthylpipérazine.

8. Composition de carburant hydrocarboné selon l'une des revendications 1 à 7, dans laquelle on fait réagir l'acide succinimique substitué par un hydrocarbyle ou un dérivé de celui-ci avec l'amine secondaire à une température de 90 à 180°C.

9. Composition de carburant hydrocarboné selon l'une des revendications précédentes dans laquelle le carburant hydrocarboné comprend une fraction hydrocarbonée qui boue dans la gamme d'ébullition de l'essence.

10. Composition de carburant hydrocarboné selon l'une des revendications 1 à 9, dans laquelle le carburant hydrocarboné comprend une fraction hydrocarbonée qui boue dans la gamme d'ébullition du diesel.
